

# UNITED STATES PATENT OFFICE.

JAMES S. PATTY, OF CHICAGO, ILLINOIS, ASSIGNOR TO CHADELOID CHEMICAL COMPANY, OF NEW YORK, N. Y., A CORPORATION OF WEST VIRGINIA.

## PAINT AND VARNISH SOLVENT.

1,235,721.

Specification of Letters Patent.

Patented Aug. 7, 1917.

No Drawing. Application filed June 13, 1912, Serial No. 703,522. Renewed June 11, 1917. Serial No. 174,172.

To all whom it may concern:

Be it known that I, JAMES S. PATTY, a citizen of the United States, and a resident of the city of Chicago, county of Cook, and 5 State of Illinois, have invented certain new and useful Improvements in Paint and Varnish Solvents, of which the following is a specification.

This invention relates to paint and varnish solvents, and is designed to provide a compound which will, when applied to the article to be cleansed, retain its liquid state for a sufficient time to entirely remove the varnish or paint.

15 It has been found that the best known solvents for paint or varnish are alcohol ( $C_2H_5OH$ ), and benzol or impure benzene ( $C_6H_6$ ). These elements, separately or in compound, preferably the latter, constitute 20 solvents for any paint or varnish.

It has been found, however, that benzol and alcohol, having very rapid evaporating or volatilizing qualities, are transformed into a gas or vapor prior to the entire removal of the paint from the surface upon 25 which they are acting. It is therefore desirable to add an element or elements which will overcome this rapid evaporating characteristic of the benzol and alcohol. Ethyl 30 or methyl palmitate has been found to overcome this rapid evaporating characteristic of benzol and alcohol, when mixed therewith; but inasmuch as the palmitate crystallizes out when placed in solution in alcohol, it is desirable to so treat the palmitate 35 that the same will not crystallize out when mixed with alcohol.

Therefore the palmitate is heated with an oily substance such as a fat or an oil, preferably sperm oil, paraffin oil, or both. This oil acts upon the palmitate to produce a mixture which, when added to the benzol and alcohol solution, will prevent the crystallization of the palmitate.

45 Furthermore, in order to add to the cutting qualities of the mixture and also to aid in retaining the palmitate in solution, calcium phenolate, phenyl salicylate, or both are then added to the mixture.

The elements heretofore described are 50 compounded in the following manner and proportions:

Primarily the benzol and alcohol are mixed and the ethyl or methyl palmitate is heated with sperm oil or paraffin oil, or both, 55 and then mixed with the mixture of benzol and alcohol. The calcium phenolate or phenyl, salicylate, or both, are then added to the mixture.

|                        |                           |    |
|------------------------|---------------------------|----|
| Benzol ( $C_6H_6$ )    | Four quarts               | 60 |
| Alcohol ( $C_2H_5OH$ ) | Five quarts               |    |
| Ethyl } palmitate      | One pound                 |    |
| Methyl } palmitate     | Four ounces               | 65 |
| Sperm oil              | Four ounces               |    |
| or                     |                           |    |
| Paraffin oil           | Four ounces               |    |
| Calcium phenolate      | { One and one-half pounds |    |
| or                     |                           |    |
| Phenyl salicylate      | { One and one-half pounds | 70 |

Should the sperm oil and paraffin oil both be used in the compound, only two ounces of each are used, and if the calcium phenolate and the phenyl salicylate are both used, 75 only three-quarters of a pound of each are placed in the mixture.

Having described my invention, what I claim as new and desire to secure by Letters Patent, is:

1. A compound of the class described comprising a solvent, an alkyl palmitate, and an oil, substantially as described.
2. A compound of the class described comprising a solvent, an alkyl palmitate, an oil, 85 and a phenol compound, substantially as described.
3. A compound of the class described comprising benzol; alcohol; an alkyl palmitate; an oil; and a phenol compound, substantially 90 as described.

In testimony whereof I have signed my name to this specification in the presence of two subscribing witnesses.

JAMES S. PATTY.

Witnesses:

JOSHUA R. H. POTTS,  
BRAYTON G. RICHARDS.